

## 1

3,252,801

PHOTOGRAPHIC EMULSIONS, LAYERS  
AND ELEMENTS

Abraham Bernard Cohen, Springfield, and Comer Drake Shacklett, Roselle, N.J., assignors to E. I. du Pont de Nemours and Company, Wilmington, Del., a corporation of Delaware

No Drawing. Filed July 10, 1961, Ser. No. 122,653  
15 Claims. (Cl. 96—114)

This invention relates to improved photographic silver halide emulsions, emulsion layers, and film elements embodying the same which are useful for continuous tone reproduction in the graphic arts industry.

Photographic films for use in the graphic arts should have good dimensional stability so that when several films are overlaid, as is customary in color reproduction, these films will be in register, i.e., in exact correspondence. To achieve a high degree of dimensional stability the photographic emulsions are often coated on glass plates. More recently, hydrophobic film bases, e.g., polyethylene terephthalate, have been used for these purposes in place of glass but the base does not solve emulsion shortcomings.

An undesirable characteristic of presently available graphic arts films is the change in image optical density which occurs from the wet to dry state. In practical use, it is usually desirable to develop the film to the required optical density as determined by inspection or in a densitometer while the film is wet; then to stop the development. This is not an accurate method because of the inherent optical density changes that occur on drying and it is often necessary to run a development series to obtain a single negative with a desired optical density balance. Moreover, the magnitude of change in wet-to-dry densities will vary with drying conditions. The previous methods are, of course, costly and time consuming.

A desirable characteristic of graphic arts films is their ability to be reduced in image density after development by mechanically removing a portion of the silver image in a controlled fashion by means of a knife, a process commonly referred to as "knife etching." Unlike chemical etching, the cohesive and adhesive properties of the binder play a vital role in determining the degree of control possible in "knife etching" and the freedom from flaking, cracking, or anchorage failure.

Attempts have been made to substitute synthetic binders for gelatin in order to improve its characteristics for graphic arts uses, but these have been only partially successful due to the unique photographic and colloid-chemical properties of gelatin as a binder. Improvements in one property are usually at the expense of another and often more important property. Bolton U.S. Patent 2,495,918, for example, suggests replacing the gelatin in a gelatino-silver halide emulsion with a poly-N-vinyl-lactam such as poly-N-vinylcaprolactam. Such emulsions, while useful, do not possess the outstanding advantages which have made gelatin the protective colloid in the emulsion making art for many years. It is difficult, for instance, to coat such poly-N-vinylactam emulsions and to obtain a layer of satisfactory hardness and stability. This is particularly true when the exposed element contains the usual photographic hardeners and is placed in aqueous photographic processing solutions. Hosmer U.S. Patent 2,754,245 discloses using the interhalogen aducts of polyvinylpyrrolidone as a gelatin extender in photographic emulsions but it is difficult to control the all-important halogen content of the system with such ad-

## 2

ducts. Many other binder modifications have been suggested but none of these provide a proper balance between the major physical and photographic properties required in graphic arts films.

5 An object of this invention is to provide a unique photographic silver halide emulsion and emulsion layer which retains the advantages of gelatin while overcoming certain disadvantages. Another object is to provide photographic emulsion layers and elements for the graphic arts industry which have improved dimensional stability. Another object is to provide photographic emulsion layers of improved dimensional stability in which the optical density of the developed image remains stable during change from a wet to a dry state. A further object is to prepare such emulsion layers which have improved "knife etchability," impact strength, and adherence to a dimensionally stable photographic film base. Still other objects will appear hereafter.

The improved gelatino-silver halide emulsions of this 20 invention comprise (1) an aqueous phase containing therein as a part of said phase (a) gelatin and (b) a water-soluble polyvinyl pyrrolidone having an average molecular weight of at least 8000 (preferably from 10,000 to 150,000) and (2) a non-aqueous phase dispersed 25 therein of water-dispersible colloidal particles (preferably of an average diameter of less than 400  $\mu$ ) of a substantially water-insoluble vinyl addition polymer of an ethylenically unsaturated monomer of molecular weight less than 250, said gelatin, polyvinyl pyrrolidone 30 and water-insoluble polymer being present in the percentages by weight from 30% to 80%, 6% to 30%, and 10% to 55%, respectively, of the total weight of the three polymeric binders. There may be present minor amounts, 35 usually less than 5% of the weight of the three binders, of various emulsion adjuvants, dispersing agents, coating aids, etc.

The novel tri-component colloid binder silver halide 40 emulsions can be made in various manners. In a preferred aspect of the invention, light-sensitive silver halide or a mixture of such halides is precipitated in an aqueous photographic gelatin solution. The resulting emulsion or dispersion retains the protective colloid and other properties of the gelatin of photographic grade. To the precipitated silver halide emulsion, which can be washed, ripened, etc., there are added suitable sensitizers and, if desired, other emulsion adjuvants, and the emulsion is digested. To the digested emulsion are added, separately or simultaneously, an aqueous solution or dispersion of the polyvinyl pyrrolidone and of the water-insoluble vinyl 50 addition polymer. After an intimate mixture is obtained, the resulting tricomponent colloid-silver halide dispersion is coated on a suitable support, e.g., a hydrophobic film base, and the coating dried. Additional gelatin can be added along with the other two colloids to provide the required amount of gelatin in the final silver halide emulsion or dispersion.

After drying, the light-sensitive silver halide layer is given a sensitometric exposure through a neutral density wedge, processed by developing, fixing, etc., and the 60 image densities are read on a conventional type of densitometer. The unique tricomponent gelatin/polyvinyl pyrrolidone/water-insoluble vinyl polymer silver halide emulsion yields a clear film which is permeable to aqueous developing and fixing solutions as is an all-gelatin film and has comparable photosensitometric properties because of the similarity in silver halide grain structure and size distribution. However, its physical, di-

dimensional and practical photographic handling properties are markedly improved. For example, the humidity coefficient of expansion and size change during processing of the light-sensitive silver halide to a silver image is markedly reduced. The optical density of the image in passing from the wet to the dry state is markedly stabilized so that a final dry optical density can be accurately predicted from a wet optical density reading. Further, the "knife etching" character of this binder is greatly improved from that of an all-gelatin film or a film containing gelatin and one of the other two colloid binding agents so that much greater etching control is possible. The drying rate of the processed, exposed film is increased, the tendency to curl at low humidities reduced, and the impact resistance and anchorage substantially improved. These combinations of properties and results are surprising and are of commercial importance in graphic arts photographic films where thick emulsion layers are often used for continuous tone reproduction.

In a preferred aspect of carrying out the invention, there can be added to the gelatino-silver halide emulsion a cationic optical sensitizing dye and a latex of the water-insoluble vinyl polymer dispersed therein by means of an amphoteric dispersing agent, preferably an amphoteric alkyliminodcarboxylate or alkylaminomonocarboxylate dispersing agent of the formula:



where R is an alkyl group of 12-18 carbon atoms, m is 0 or 1, p is 2-m and M is a cation selected from the group consisting of hydrogen, sodium, potassium and ammonium. In general, the dispersing agent is used in an amount from 0.5% to 15.0% by weight of the water-insoluble vinyl polymer.

Suitable amino acid dispersing agents are disclosed in U.S. Patent 2,816,920, Dec. 17, 1957, and are commercially available. Two of these dispersing agents of particular interest are disodium-N-tallow-beta-iminopropionate and the disodium salt of N-dodecyl-beta-iminodipropionate. In the case of the former dispersing agent, "tallow" represents a mixture of the alkyl radicals oleyl, palmityl, stearyl and myristyl in order of decreasing concentration. Non-ionic as well as cationic surfactants can be used, but best results can be obtained, especially in the case of the panchromatic silver halide emulsions, by means of the amphoteric alkyliminodcarboxylate dispersing agents described above.

The polyvinyl pyrrolidones useful in the emulsion can vary over a fairly wide range of average molecular weight but have an average molecular weight between 10,000 and 150,000. Higher average molecular weights still bring about improvements in certain characteristics of the film but haze sometimes is encountered as the molecular weight increases beyond the preferred range. With molecular weights below the preferred range, the desirable effects are less pronounced since the lower molecular weight material tends to diffuse out of the emulsion during photographic processing of the coated element.

Considerable latitude is possible in the choice of the colloid dispersion of the water-insoluble vinyl polymers, including copolymers. A preferred class are the alkyl acrylates and methacrylates, e.g., polymers and copolymers of methyl, ethyl, butyl, ethylhexyl acrylate or methyl and butyl methacrylate. Also, acrylic or methacrylic acid can be used in the preparation of useful copolymers. With most co-monomers, no more than 10 mole percent of such an acid is used in the polymerization with the other constituents so that the copolymer will remain water-insoluble. Other useful classes of vinyl monomers used to prepare water insoluble polymer and copolymer dispersions useful in accordance with this invention are the vinyl esters such as the acetate, propionate, etc.; the vinyl and vinylidene halides such as vinylidene chloride; styrene and substituted styrenes; the dienes such as

butadiene; acrylonitrile; alkenes such as ethylene or propylene and the like. The water-insoluble polymers are free from color-former nuclei or groups.

In general, the best results are obtained with vinyl monomers which yield the lowest water sensitivity and lowest modulus of elasticity. Thus, acrylates in general are preferable to methacrylates and polyethylene to polyvinylidene chloride polymers and copolymers. The vinyl polymers, in general, have an average molecular weight above 10,000.

The particle size of vinyl dispersion is important, since the intended application requires freedom from light-scattering. In general, particle sizes below the wavelength of light, i.e., below 400  $\mu$ , would be preferred. This may be controlled by techniques of emulsion polymerization known in the art such as the use of adequate concentrations of surfactants, the mode of stirring, the concentrations of reactants, temperature, rate of additions of monomers, etc.

20 In order to realize the full advantages of the improved dimensional stability of the emulsions of this invention, it is desirable to coat the emulsions on a film base support which also has adequate dimensional stability, e.g., polymethylene terephthalates, polystyrene, polycarbonates,

25 e.g., the polycarbonate of 2,2-bis-p-hydroxyphenyl propane, polyethylene terephthalate/isophthalate, etc. In general the polyester films include those prepared from highly polymerized esters of terephthalic acid and at least one glycol of the formula  $HOCH_2-W-CH_2OH$  30 where W is polymethylene or alkyl-substituted polymethylene of 0 to 8 carbons, e.g., 2,2-dimethylpropylene-1,3 or a cycloalkylene radical of 5 to 6 carbon atoms, e.g., cyclopentyl-1,3, and cyclohexyl-1,4. Polymeric films comprising up to 20 mole percent of aliphatic dicarboxylic acids based on total moles of acids, e.g., succinic, 35 glutaric, adipic, hexahydroterephthalic and sebacic acids, in addition to at least 15 mole percent terephthalic acid, are also useful.

40 The above-described polymers or copolymers may contain a number, e.g., 1 to 12 or more, of ether groups in the polymer chain. Such ether groups may be added as part of ether containing glycol derivatives or formed by side reactions during polymerization. Also the emulsions may be coated on various films and plates composed of 45 glass, metal, e.g., aluminum, various waterproof papers, cellulose derivatives, e.g., cellulose acetate, cellulose propionate, cellulose butyrate, cellulose acetate-butyrate, and cellulose nitrate; other superpolymers, e.g., nylon, polyvinyl chloride, poly(vinyl chloride co vinyl acetate), etc.

50 The polymer dispersions used in a preferred embodiment of this invention are prepared in a conventional manner, starting with a polymerizable liquid monomer. This monomer is emulsified with water by means of the dispersing agents described above, and subjected to a 55 conventional emulsion polymerization using a free radical initiator, e.g. peroxide or  $\alpha,\alpha'$ -azo bis-(isobutyronitrile). In Procedure A, to follow, there is given a description of the preparation of a particularly preferred dispersion, that of polyethylacrylate. Alternately one can use a bulk polymerization and prepare the dispersions by dispersing the molten polymer in water in the presence of a dispersing agent, such as is commonly done with polyethylene.

60 The invention will be further illustrated by, but is not intended to be limited to, the following procedures and examples wherein the coatings were evaluated as follows for their humidity coefficient of expansion, dimensional stability, knife etchability, adhesion and curl:

65 In determining humidity coefficient of expansion, a 30 inch strip of a coating is scribed with a sapphire micro-groove stylus so as to produce, near each end of the strip, fiducial marks which will be in close proximity to the fiducial marks of a calibrated Invar plate when the strip and Invar plate are brought into contact with one 70 another. The strip is then conditioned for 24 hours at 75

a constant temperature and humidity and then, while maintained at the same conditions, placed in flat contact with the Invar plate. Two Gaertner filar micrometer microscopes, having a total magnification of 100 diameters and micrometer least count  $2 \times 10^{-5}$  inches, are mounted so that measurements may be obtained by means of a graduated glass scale of distances between the fiducial marks on the coating strips and the corresponding fiducial marks on the Invar plate. The Invar plate, microscopes and coating strip are all housed in a conditioning cabinet equipped with arm ports and viewing windows. By vector addition of these distances and the known distance between the fiducial marks on the Invar plate, the distance is determined between the two fiducial marks on the strip at a known humidity. The process is repeated, with 24 hour preconditioning, to determine the distance between the strip's two fiducial marks at another known humidity. The change in length at the two humidity values divided by the average of the two lengths and divided by the difference in percent relative humidity gives the humidity coefficient of expansion. Invar is a nickel-steel alloy. Dimensional stability in terms of processing size change is determined in a very similar manner. Distance between fiducial marks is determined on a coating strip which has been conditioned under constant temperature and humidity for 24 hours. The strip is then conventionally processed and dried, conditioned at the previous constant temperature and humidity for 24 hours, and measured to determine the change in distance between fiducial marks. The processing size change is calculated by dividing this change in distance by the average distance.

Knife etching is a subjective test wherein the etcher rates various materials on the basis of his ability, by means of a knife, to produce smooth gradations in density from high to low from an area having an original high image density. Chipping, cracking, flaking, adhesive failure etc., would cause a poor rating in terms of "knife etchability."

Values of impact strength under various conditions were obtained using an apparatus similar to that described by R. D. Spangler and E. B. Cooper, Journal of Applied Physics, vol. 28, No. 3, March 1957, pages 329-333. In this apparatus, the measured quantity is the amount of energy absorbed by a film when a steel ball is projected through it. By means of photoelectric cells, the velocity of a steel ball in free flight can be compared with its velocity after having passed through the film being examined.

Dry adhesion of emulsion to the support was measured by the common test wherein cross-hatched lines are cut through the emulsion and a piece of pressure-sensitive tape is applied to an emulsion surface and then rapidly pulled off. Removal of a part of the emulsion from the base indicates inferior anchorage. Wet anchorage can be determined similarly after normal photographic processing, by determining the tendency of the wet emulsion to lift off the base when a force is applied tangentially at the edge of the cross hatched lines.

Curl was measured by determining the weight required to restore a 10" x 12" sheet of film conditioned at 20% R.H. and 75° F. to a flat condition.

#### PROCEDURE A

A 22-liter fluted reaction pot was equipped with a thermometer, anchor stirrer, three-neck adapter containing a gas inlet tube and two reflux condensers. The system was purged with nitrogen for 10 to 20 min. and maintained under a positive nitrogen pressure throughout the polymerization. To the pot were added 10 liters of distilled water, 484 g. of disodium-N-tallow- $\beta$ -iminodipropionate flakes (96%) and 50 g. of gelatin (used as a thermal stabilizer) with 1040 ml. of distilled water. The mixture was allowed to soak at room temperature with

moderate agitation for 10-15 minutes. The stirred reaction mixture was heated by a water bath to 50-55° C. for 15-20 min. to effect solution. To the aqueous solution in the pot was added 3300 g. of ethyl acrylate (from which the polymerization inhibitor had been removed by extraction with alkali). The stirred reaction mixture was heated by a water bath to 80-85° C., held for 10 min. in this temperature range and cooled to 75° C. To the reaction mixture was added 60 ml. of a 30% by weight aqueous solution of hydrogen peroxide and the temperature was held at 75° C. until the polymerization initiated. After the initial exothermic reaction had subsided (note: moderated with cold water as required to control excessive foaming), 1700 g. of ethyl acrylate were added to the pot. The bath temperature was adjusted to  $75 \pm 3$ ° C. and 19 ml. of a 30% by weight aqueous solution of hydrogen peroxide was added. After the second stage of the polymerization had subsided, the temperature was raised to 80-85° C. and held in this range for 2 hours. The dispersion was then heated to 90° C., held for 10 min. and steam distilled for 1 to 2 hours to remove any residual monomer. The dispersion was cooled to about 50° C. and filtered through felt to remove any residue. The composition by weight of the dispersion made by this procedure is 30% polyethyl acrylate and 2.79% disodium-N-tallow- $\beta$ -iminodipropionate.

#### PROCEDURE B

A 22 liter fluted pot was equipped as described in Procedure A and purged with nitrogen in the same manner. To the pot were added 8 liters of distilled water and 16.7 g. of a high molecular weight polyacrylamide (thermal stabilizer), which was added slowly through a long stem funnel of narrow bore and washed in with 2.5 liters of distilled water. The mixture was stirred for 2 to 3 hours at room temperature to effect solution. To the solution of polyacrylamide in the pot were added 667 g. of a 30% by weight aqueous solution of sodium lauryl sulfate which was washed in with 400 ml. of distilled water, 1000 g. of ethyl acrylate (from which the polymerization inhibitor had been removed by extraction with alkali). The stirred reaction mixture was heated by a water bath to 80-85° C.; for 10 min. in this temperature range and cooled to 75° C. To the reaction mixture was added 16 ml. of a 30% by weight aqueous solution of hydrogen peroxide and the temperature was held at 75° C. until the polymerization initiated. After the initial exothermic reaction had subsided (note: moderated with cold water as required to control excessive foaming), 1000 g. of ethyl acrylate and 16 ml. of a 30% by weight aqueous solution of hydrogen peroxide were added and this process was repeated until the total amounts of ethyl acrylate and hydrogen peroxide added were respectively 5000 g. and 80 ml. After the fifth stage of the polymerization had subsided, the dispersion was treated as shown in Procedure A to complete the polymerization and remove the residual monomer. The composition by weight of the dispersion made by this procedure is 30% polyethyl acrylate and 1.2% sodium lauryl sulfate.

#### PROCEDURE C

A 22-liter fluted pot was equipped as described in Procedure A and purged with nitrogen in the same manner. A solution of high molecular weight polyacrylamide (thermal stabilizer) was prepared as described in Procedure B. To the solution of polyacrylamide in the pot were added 667 g. of a 30% by weight aqueous isopropanol solution of a surfactant of the formula



which was washed in with 400 ml. of distilled water. A two stage polymerization was carried out as described in Procedure A except that butyl acrylate was used in place of ethyl acrylate. The composition by weight of

the dispersion made by this procedure is 30% polybutyl acrylate and 1.2% polyether sulfate surfactant.

#### PROCEDURE D

Procedure C was essentially repeated except that 800 g. of a 25% by weight aqueous solution of "Tamol" 731 (registered trade name, Rohm & Haas, defined by Haynes, Chemical Trade Names and Commercial Synonyms, 2nd edition, 1955, Van Nostrand and Co., New York, as the "sodium salt of a carboxylated polyelectrolyte") which was washed in with 267 ml. of distilled water was used in place of the sodium salt of a polyether sulfate surfactant. A two-stage polymerization was carried out as described in Procedure A except that methyl methacrylate was used in place of ethyl acrylate. The composition by weight of the dispersion made by this procedure is 30% polymethyl methacrylate and 1.2% sodium salt of carboxylated polyelectrolyte.

#### PROCEDURE E

Procedure C was essentially repeated except that 200 g. of sodium stearate which was washed in with 867 ml. of distilled water was used in place of the sodium salt of an alkyl aryl polyether sulfate. A two stage polymerization was carried out as described in Procedure A except that styrene was used in place of ethyl acrylate and the bath temperature was 80° C. instead of 75° C. The composition by weight of the dispersion made by this procedure is 30% polystyrene and 1.2% sodium stearate.

#### PROCEDURE F

Procedure A was essentially repeated except that 716 g. of a 28% by weight aqueous solution of a surfactant of the formula



which was washed in with 714 ml. of distilled water, was used in place of disodium-N-tallow- $\beta$ -iminodipropionate. A mixture of monomers consisting of 3500 g. of vinylidene chloride and 1500 g. of 2-ethylhexyl acrylate was used in place of ethyl acrylate.

An aqueous solution of 33.3 g. of ammonium persulfate dissolved in 100 ml. of distilled water and an aqueous solution of 16.7 g. of sodium metabisulfite dissolved in 50 ml. of water were used in place of hydrogen peroxide. The polymerization was carried out at 25-30° C. instead of at 75° C. The composition by weight of the dispersion made by this procedure is 21%/9% co-polyvinylidene chloride/2-ethylhexyl acrylate and 1.2% sodium salt of the alkyl aryl polyether sulfonate surfactant.

#### PROCEDURE G

Procedure A was essentially repeated except that 333 g. of isoctyl phenyl polyethoxy ethanol which was washed in with 1190 ml. of distilled water was used in place of disodium-N-tallow- $\beta$ -iminodipropionate. The composition by weight of the dispersion made by this procedure is 30% polyethyl acrylate and 2% isoctylphenylpolyethoxy ethanol.

#### PROCEDURE H

To a 2-liter beaker was added 600 g. of pellets of a commercially available polyethylene having a melting point in the range of 101-105° C. and a viscosity at 5 140° C. of 160 cps. The material was slowly melted with intermittent stirring and raised to a temperature of 130° C. at which time 135 g. of oleic acid was added with thorough stirring. At the end of the addition there was a 5° lowering of temperature. After the temperature was again raised to 130°, 120 g. of distilled morpholine was stirred in and the temperature (which had dropped to about 122°) was raised to 127°. Over a period of 3-4 minutes the liquid was added, with vigorous stirring, to a 4-liter beaker containing 2800 g. of 10 distilled water which had been preheated to a temperature range of 97°-99° C. The dispersion thus prepared was allowed to cool slowly to 87°, then cooled in cold water and finally ice water to 30° C. It was then filtered through 15 felt to remove any hard residue. The composition by 20 weight of the dispersion made by this procedure is 17.7% polyethylene and 4.9% morpholine oleate.

#### Example I

25 A photographic emulsion was precipitated and ripened in a conventional way and freed of unwanted soluble salts by a coagulation and wash procedure taught in Example I of Moede, U.S. 2,772,165. The silver halide composition was 96.3 mole percent AgBr and 3.7 mole percent 30 AgI in the presence of 14.7 g. of gelatin per mole. The coagulated emulsion was redispersed in water in the presence of additional gelatin, digested at elevated temperatures in the presence of conventional sulfur sensitizers, 35 cooled and stabilized with post-sensitization additives common in the art such as additional halide, antifoggants etc. It was then divided into seven equal portions and to six of these portions there was added, with good stirring additional gelatin, a 40% by weight aqueous solution of 40 poly-N-vinyl pyrrolidone (PVP) having an average molecular weight of 40,000 and an aqueous dispersion containing 30% by weight polyethyl acrylate as was prepared under Procedure A. The final binder compositions in each portion were as shown in Table I. To portion No. 1, 45 serving as a control, only gelatin was added.

These emulsions were applied at a silver halide coating weight of 110 mg./dm.<sup>2</sup> (calculated as silver bromide) onto 7-mil thick polyethylene terephthalate film base bearing a substratum of a vinylidene chloride/methyl acrylate/itaconic acid copolymer such as is described in Example 50 IV of Alles patent, U.S. 2,779,684 and over this a second substratum containing 0.5 mg./dm.<sup>2</sup> of gelatin. The emulsions were then evaluated for various physical characteristics by tests already described using a relative scale in which A represents the most desirable and D the least desirable relative rating for the intended applications. 55 Such letters indicate a subjective averaging of numerical values obtained under a variety of conditions. Results are 60 shown in Table I.

TABLE I.—BINDER COMPOSITION PHOTOGRAPHIC PROPERTIES

| No.    | Percent Gelatin | Percent PVP | Percent Polyethyl Acrylate Dispersion | Relative Speed | Contrast | Wet-to-Dry Density Change | Knife Etching | Curl   | Impact Resistance | Dimensional Stability | Anchorage | Drying Rate |
|--------|-----------------|-------------|---------------------------------------|----------------|----------|---------------------------|---------------|--------|-------------------|-----------------------|-----------|-------------|
| 1----- | 100             | 0           | 0                                     | 1.0            | 0.8      | - .14                     | C-----        | D----- | C-----            | C-----                | D-----    | C           |
| 2----- | 73.5            | 16.5        | 10                                    | 2.0            | 1.0      | + .09                     | A-----        | C----- | C-----            | C-----                | B-----    | B           |
| 3----- | 55.5            | 16.5        | 28                                    | 2.2            | 1.1      | + .06                     | A-----        | B----- | B-----            | B-----                | A-----    | B           |
| 4----- | 55.5            | 5.5         | 39                                    | 1.5            | .9       | - .14                     | D-----        | A----- | A-----            | A-----                | A-----    | A           |
| 5----- | 50              | 13          | 37                                    | 2.0            | 1.0      | 0                         | B-----        | A----- | A-----            | A-----                | A-----    | A           |
| 6----- | 40              | 8.5         | 51.5                                  | 1.9            | .9       | - .09                     | C-----        | A----- | A-----            | A-----                | A-----    | A           |
| 7----- | 55.5            | 22          | 22.5                                  | 2.9            | 1.3      | + .20                     | A-----        | B----- | B-----            | B-----                | A-----    | A           |

In Table I, the sensitometric data was obtained from film strip samples of the coatings which were given a 20 second, intensity-scale, sensitometric, step-wedge exposure to a white light tungsten source. The exposure in each successive step increased by the factor of the square-root of two. The exposed film strips were developed for 3 minutes in a developer of the following composition to determine its sensitometric characteristics:

and F. To the sixth portion, serving as a control, only gelatin was added. Upon coating and evaluation as described in Example I, improvement were obtained, shown in Table II, similar to those Example I except that the balance of certain properties varied with the particular dispersion used.

The polystyrene sample had an average particle size greater than the other polymers.

TABLE II

| Water Insoluble Vinyl Polymer                        | Dispersing Agent                    | Relative Speed | Wet-to-dry Density Change | Knife Etching | Dimensional Stability | Curl   | Impact Strength | Anchorage |
|------------------------------------------------------|-------------------------------------|----------------|---------------------------|---------------|-----------------------|--------|-----------------|-----------|
| Polyethyl acrylate.....                              | Alkyl imino-dipropionate.....       | 2.2            | +.09                      | B.....        | B.....                | B..... | B.....          | A.....    |
| Polybutyl acrylate.....                              | Alkyl aryl polyether sulfate.....   | 2.5            | +.02                      | B.....        | A.....                | A..... | A.....          | A.....    |
| Polymethyl methacrylate.....                         | Polycarboxylate.....                | 2.5            | +.02                      | A.....        | C.....                | C..... | B.....          | C.....    |
| Polystyrene.....                                     | Sodium stearate.....                | 2.5            | -.11                      | D.....        | B.....                | C..... | C.....          | C.....    |
| Copolyvinylidene chloride/2-ethylhexyl acrylate..... | Alkyl aryl polyether sulfonate..... | 2.1            | +.07                      | A.....        | B.....                | A..... | A.....          | A.....    |
| None (Control).....                                  | None.....                           | 1.0            | -.14                      | C.....        | C.....                | D..... | C.....          | D.....    |

## G.

|                                                         |      |    |
|---------------------------------------------------------|------|----|
| Monomethyl-p-aminophenol sulfate .....                  | 2.5  | 25 |
| Na <sub>2</sub> SO <sub>3</sub> , desiccated .....      | 50.0 | 25 |
| Hydroquinone .....                                      | 2.5  | 25 |
| Na <sub>2</sub> CO <sub>3</sub> .H <sub>2</sub> O ..... | 24.0 | 25 |
| Borax .....                                             | 14.0 | 25 |
| KBr .....                                               | 0.5  | 25 |
| Water to make 1.0 liter.                                |      | 30 |

## Example III

An emulsion was prepared according to the procedure of Example I and divided into three parts. To each part was added a polyethyl acrylate dispersion prepared according to Procedure A and a solution of polyvinyl pyrrolidone of varying molecular weights. Evaluation was carried out as described in Example I. Binder compositions and resulting properties are shown in Table III.

TABLE III

| Percent Gelatin | Percent PVP | Percent Polyethyl Acrylate | Approx. Mol. Wt. PVP | Speed | Wet-to-dry Density Change | Knife Etching | Dimensional Stability | Impact Resistance | Curl  |
|-----------------|-------------|----------------------------|----------------------|-------|---------------------------|---------------|-----------------------|-------------------|-------|
| 100.0           | -----       | -----                      | -----                | 1.0   | -.14                      | -----         | -----                 | -----             | ----- |
| 55.5            | 11          | 33                         | 10,000               | 1.8   | -.09                      | B             | C                     | C                 | C     |
| 55.5            | 16.5        | 28                         | 40,000               | 2.2   | +.06                      | A             | B                     | B                 | B     |
| 55.5            | 22          | 22.5                       | 350,000              | 2.9   | +.03                      | C             | B                     | C                 | C     |

After development, the strips were treated in a conventional acid hardening and fixing bath containing 153 g. anhydrous Na<sub>2</sub>S<sub>2</sub>O<sub>3</sub> per liter, washed in tap water and dried in a conventional manner. Optical densities of the film strips were read at each exposure step on a Western Electric RA-1100C densitometer, the readings being made both at the start of the drying period when the films were wet and at the end of the drying period. The wet-to-dry density changes recorded in the tables correspond to dry optical densities of approximately 2.0. A negative or positive sign for this density change indicates a loss or gain, respectively, of density on drying. All the films in this example, including the control with an all gelatin binder, had low fog.

These results indicate the binder composition of this invention yields improvements in most of the critical properties required in photographic films, in particular for those used in graphic arts applications. As can be noted, different balances of properties are attainable for different ratios of the three binder components with the coating from emulsion portion No. 5 representing the best overall balance.

## Example II

An emulsion was prepared as in Example I and was divided into six portions. To each of five portions were added a 40% by weight aqueous solution of polyvinyl pyrrolidone (M.W.=40,000) and an aqueous dispersion containing 30% by weight of various water insoluble vinyl polymers so that the final binder solids composition by weight would be 55.5/16.5/28, gelatin/polyvinyl pyrrolidone/dispersed polymer. The dispersions used were prepared, respectively, according to Procedures A, C, D, E,

45 While the molecular weight of the polyvinyl pyrrolidone appears to have a quantitative effect favoring an intermediate molecular weight, improvements are possible over a wide range of molecular weights provided the polyvinyl pyrrolidone is water soluble and the concentrations of latex and gelatin are properly balanced for the particular polyvinyl pyrrolidone. The haze level was considered undesirable in the coating employing the polyvinyl pyrrolidone of 350,000 molecular weight. For some less critical applications this haze level may be tolerable.

## Example IV

55 An emulsion was prepared as in Example II, half of which contained gelatin as the only binder material, while the other half was treated, as was emulsion portion No. 1 of Example II, by adding the same amounts of polyvinyl pyrrolidone solution and of a polyethyl acrylate dispersion prepared according to Procedure A. The final binder solids composition by weight was, therefore, 55.5/16.5/28, gelatin/polyvinyl pyrrolidone/polyethyl acrylate.

60 A similar but higher contrast emulsion was prepared with variations of ripening and digestion conditions in the manner customary in the art. As in the paragraph above, half of this emulsion contained gelatin as the only binder material, while the other half was treated by adding the same amounts of a polyvinyl pyrrolidone solution and of a polyethyl acrylate dispersion.

65 The four emulsions were coated as in Example I except that the film base support had coated on the reverse side an antihalation backing containing no silver halide but with binder composition and coating weight identi-

cal to the emulsion binder. Evaluation as in Example I gave the results shown below in Table IV.

TABLE IV

| Coating               | Percent Gelatin | Percent PVP | Percent Polyethyl Acrylate | Relative Speed | Contrast | Wet-to-Dry Density Change | Knife Etching | Humidity Coefficient of Expansion $\times 10^5$ | Impact Strength | Anchorage |
|-----------------------|-----------------|-------------|----------------------------|----------------|----------|---------------------------|---------------|-------------------------------------------------|-----------------|-----------|
| Low Contrast Control  | 100             |             |                            | 1.0            | 1.0      | -.10                      | C-----        | 3.5                                             | D-----          | B.        |
| Low Contrast Coating  | 55.5            | 16.5        | 28                         | 2.0            | 1.0      | +.01                      | A-----        | 2.7                                             | A-----          | A.        |
| High Contrast Control | 100             |             |                            | 1.0            | 1.4      | -.12                      | C-----        | 3.5                                             | D-----          | B.        |
| High Contrast Coating | 55.5            | 16.5        | 28                         | 1.5            | 1.4      | 0                         | A-----        | 2.7                                             | A-----          | A.        |

### Example V

An emulsion was prepared similar to that in Example I except that a symmetrical thiocarbocyanine ethiodide optical sensitizing dye was added during digestion to render it panchromatic. The emulsion was divided into three portions and an aqueous solution of polyvinyl pyrrolidone and an aqueous dispersion of polyethyl acrylate were added to each portion. The final binder composition of the first portion was identical to that of the first portion of Example II wherein the polyethyl acrylate polymer was dispersed with an amphoteric dispersing agent, disodium-N-tallow-beta-iminodipropionate (Procedure A). The second emulsion portion was the same except that the polyethyl acrylate was dispersed with an anionic surfactant, sodium lauryl sulfate (Procedure B). The third emulsion portion was the same except that the polyethyl acrylate was dispersed with a nonionic agent, isoctylphenyl polyethoxyethanol (Procedure G).

The three emulsions were coated as in Example I except that the polyethylene terephthalate film base support bore only the single copolymeric substratum (i.e., the "second substratum containing 0.5 mg./dm.<sup>2</sup> of gelatin" was absent), and had good anchorage and gave results similar to Examples I-IV.

### Example VI

The coating from emulsion portion No. 5 of Example I was essentially duplicated except that the dispersed water-insoluble vinyl polymer used in the present example was polyethylene, prepared as described in Procedure H. This coating, when compared with an all gelatin binder control by processing both films as described in Example I, was found to exhibit less wet-to-dry density change and improved dimensional stability.

In addition to the polymeric materials specifically disclosed in the examples, there are various other materials which can be used to make approximately equivalent dispersions, e.g., polybutyl acrylate and copolymers of ethyl acrylate, butyl acrylate or ethylhexyl acrylate, and acrylic acid containing less than about 10 mole percent of acrylic acid. These polymers are physically fairly soft. Other polymers are useful equivalents in the practice of this invention but, because of being relatively harder, they are considered to be less desirable materials. Among these polymers, listed in order of decreasing physical hardness, are polymethyl acrylate and polyethyl methacrylate.

The present invention is not limited to the use of a particular film base support as the emulsions may be coated on various films and plates composed of glass, metal, e.g. aluminum, cellulose derivatives, e.g., cellulose acetate, propionate, butyrate, acetate-butyrate, and nitrate; superpolymers, e.g., nylon, polyvinyl chloride, poly(vinyl chloride co-vinyl acetate), polystyrene and polyesters such as the poly/methylene terephthalates, polycarbonates, e.g., the polycarbonate of 2,2-bis-p-hydroxyphenyl propane, polyethylene terephthalate/isophthalate, etc.

Other useful polyester films include those prepared from highly polymerized esters of terephthalic acid and at least one glycol of the formula  $\text{HOCH}_2-\text{W}-\text{CH}_2\text{OH}$  where W is polymethylene or alkyl substituted polymethyl-

ene of 0 to 8 carbons, e.g., 2,2-dimethylpropylene-1,3 or a cycloalkylene radical of 5 to 6 carbon atoms, e.g., cyclo-

pentyl-1,3, and cyclohexyl-1,4. Films comprising up to 15 20 mole percent of aliphatic dicarboxylic acids based on total moles of acids, e.g., succinic, glutaric, adipic, hexahydroterephthalic and sebatic acids in addition to at least 15 mole percent terephthalic acid are also useful. The 20 above described polymers may contain a number (e.g., 1 to 12 or more) of ether groups in the polymer chain. Such ether groups may be added as part of ether containing glycol derivatives or formed by side reactions during polymerization.

Of course, various sublayers may be present to anchor 25 the layer to the base as is common in photographic film and plate manufacture. Also, various other auxiliary layers may be employed such as antiabrasion layers and antihalation backing or undercoat layers.

The emulsions may be modified by the addition of 30 general emulsion sensitizers, e.g., alkyl thiourea, phenyl isothiocyanate, sodium thiosulfate, and alkyl isothiocyanate; metal compounds e.g., of gold, platinum, palladium, iridium, rhodium, mercury, cadmium etc.; antifogging 35 agents, e.g., 2-mercaptopbenzothiazole, 1-phenyl-5-mercaptopbenzothiazole, benzotriazole, triazindene, tetrazindene and 5-nitrobenzimidazole; sensitizing dyes; color formers (which might, alternatively, be in the developer solution); hardeners, e.g., formaldehyde and other aliphatic aldehydes, dimethylol urea, trimethylol melamine; chrome alum and other chromium compounds, coating aids, image color modifiers, brightening agents, colorants, e.g. pigments, matting agents and other emulsion adjuvants.

Photographic requirements of graphic arts emulsions 45 are generally best met by silver halides in which the predominant halide is bromide. Up to 10 mole percent iodide is added to vary the photographic behavior as well as the usual chemical sensitizers and optical sensitizing dyes. However, the unique binder advantages of this 50 invention such as wet-to-dry density stability, knife etchability, impact resistance, dimensional stability, and anchorage to the support are also applicable in varying degrees to other halides over a wide range of compositions including silver chloride, chloro-bromide and iodo chloro-bromide emulsions.

55 While these elements have their greatest usefulness in graphic art applications, many of the unique properties would be advantageous in other photographic films, e.g., cine, X-ray, portrait and color films. They could be used in monolayer or multilayer coated products. In 60 general, these elements would be applicable to special processing variations used with conventional films, e.g. for dye inhibition films or preparing planographic printing plates.

This invention has the advantage of providing superior 65 photographic emulsions for the manufacture of films having improved physical properties and improved wet-to-dry optical density stability of the developed image. Films made according to the present invention do not suffer the disadvantage of loss of optical density of the 70 developed image during drying of the film. Among the improved physical properties, dimensional stability is particularly significant but improved flexibility and improved anchorage are also important. These advantages have been achieved without sacrifice in sensitometric or other 75 physical properties of the film; in fact, photographic

speed, as can be seen in Ex. I, is significantly increased. The preferred classes of ionic dispersing agents disclosed in this invention make possible the formation of polymer particles of sufficiently small size to provide a transparent film when mixed with gelatin, coated and dried.

The particularly preferred amphoteric dispersing agents used in the panchromatic emulsions, in contrast to the anionic and cationic surfactants used in previously disclosed products, do not interfere with dye sensitization. A further advantage is the simplicity of the process of this invention; since the additions are in the form of aqueous solutions and dispersions, the process can be carried out simply and economically on a commercial scale with no need for elaborate equipment such as solvent recovery systems.

Polymers are often incompatible and, therefore, mixtures of two or three polymers cause difficulties where clarity is desired, as in photographic films. There are no reliable rules known in polymer science for predicting when compatibility will occur or what balance of properties the final polymer mixture will have. According to the present invention, however, applicants have provided a mixture of three different polymers and have found them to be compatible and to give photographic emulsions having excellent optical clarity as well as other useful photographic and physical properties.

We claim:

1. A photographic gelatino-silver halide emulsion comprising (1) an aqueous phase containing therein as a part of said phase (a) gelatin and (b) a water-soluble polyvinyl pyrrolidone having an average molecular weight of at least 8,000 and (2) a dispersion therein of water-dispersible colloidal particles of a substantially water-insoluble vinyl addition polymer of an ethylenically unsaturated monomer of molecular weight less than 250, said gelatin, polyvinyl pyrrolidone and water-insoluble polymer being present in the percentages by weight from 30% to 80%, 6% to 30% and 10% to 55%, respectively, of the total weight of the three polymeric binders.

2. An emulsion according to claim 1 wherein said colloidal particles have an average diameter of less than 400  $\mu$  and an average molecular weight above 10,000.

3. A photographic emulsion layer formed from an emulsion defined in claim 1.

4. An emulsion layer according to claim 3 wherein said polyvinyl pyrrolidone is poly-N-vinyl pyrrolidone having an average molecular weight from 10,000 to 150,000.

5. An emulsion layer according to claim 3 wherein the sum of the light absorbed and scattered by the combination of the three polymeric binder components in the absence of silver and silver salts corresponds to an optical density of not more than 0.1.

6. An emulsion layer according to claim 3 wherein said water-insoluble vinyl addition polymer is a polyalkyl acrylate.

7. An emulsion layer according to claim 3 wherein the silver halides is 10 to 99 mole percent bromide, 0 to 90

mole percent chloride, and 0 to 10 mole percent iodide.

8. An emulsion layer according to claim 3 containing an amphoteric dispersing agent of the formula:



5 where R is an alkyl group of 12-18 carbons,  $m$  is one of the numbers 0 and 1,  $p$  is  $2-m$  and M is a cation selected from the group consisting of hydrogen, sodium, potassium and ammonium.

10 9. An emulsion layer according to claim 3 wherein said halide is silver bromoiodide.

10 10. A photographic film comprising a film support bearing an emulsion layer as defined in claim 3.

11 11. A photographic film comprising a dimensionally-stable hydrophobic film support bearing on one surface 15 an emulsion layer as defined in claim 3.

12 12. A photographic film according to claim 10 having on the other surface an antihalation, anti-curl backing layer.

20 13. A process for preparing a modified gelatino-silver halide emulsion which comprises adding to a silver halide emulsion precipitated in gelatin, after digestion, an aqueous solution of a water-soluble poly-N-vinyl pyrrolidone and an aqueous dispersion of colloidal particles of a substantially water-insoluble vinyl addition polymer of an unsaturated monomer of molecular weight less than 250 to form an emulsion containing said polymeric components in the percentages by weight of 30% to 80%, 6% to 30%, and 10% to 55%, respectively, of the total weight 30 of said components.

14. A process according to claim 13 wherein the polyvinyl-N-pyrrolidone and the water-insoluble polymer are added separately.

35 15. A process according to claim 13 wherein the polyvinyl-N-pyrrolidone and the water-insoluble polymer are admixed and the mixture added to the gelatino-silver halide emulsion.

#### References Cited by the Examiner

##### UNITED STATES PATENTS

|           |         |                  |       |        |
|-----------|---------|------------------|-------|--------|
| 2,698,794 | 1/1955  | Godowsky         | ----- | 96—98  |
| 2,964,405 | 12/1960 | Talbot et al.    | ----- | 96—114 |
| 3,000,740 | 9/1961  | De Belder et al. | ----- | 96—114 |
| 3,000,741 | 9/1961  | De Pauw et al.   | ----- | 96—114 |

##### FOREIGN PATENTS

|         |        |                |  |
|---------|--------|----------------|--|
| 536,673 | 4/1955 | Belgium.       |  |
| 793,549 | 4/1958 | Great Britain. |  |

##### OTHER REFERENCES

Evva: Chemical Abstracts, vol. 52, pages 8808-9 (1958).

NORMAN G. TORCHIN, Primary Examiner.

55 HAROLD N. BURSTEIN, Examiner.

J. T. BROWN, Assistant Examiner.